

## 1

3,505,183

PROCESS AND COMPOSITIONS FOR  
ELECTROPLATING CHROMIUM

Edgar J. Seyb, Jr., 23061 Norwood, Oak Park, Mich. 48237; Hyman Chessin, 7146 Heather Heath Lane, Birmingham, Mich. 48010; and Fred Aoun, 1999 E. Saratoga, Ferndale, Mich. 48220

No Drawing. Continuation-in-part of application Ser. No. 421,600, Dec. 28, 1964. This application Mar. 4, 1968, Ser. No. 709,874

Int. Cl. C23b 5/06, 5/46

U.S. Cl. 204—51

28 Claims

## ABSTRACT OF THE DISCLOSURE

A bright decorative plating process for electroplating chromium on a basis metal, characterized by high coverage and throwing power, utilizes a chromic acid plating bath containing the anion of a halogenated organic carboxylic acid having at least three carbon atoms. The baths are of high  $\text{CrO}_3$  to catalyst ratio, e.g. 125–550:1. They may be of the self-regulating type. The halogenated carboxylic acid anion may be added by introducing into the bath the acid itself, or a soluble salt of the acid, or the acid anhydride. The anions of the halogenated aliphatic dicarboxylic acids such as 3,4-dichloroadipic acid and 2,2-dichlorosuccinic acid are preferred. The concentration of the halogenated carboxylic acid anion is preferably from 25 to 100 grams per liter, but higher concentration up to saturation may be used.

This application is a continuation-in-part of application Ser. No. 421,600, filed Dec. 28, 1964, now abandoned.

This invention relates to a novel process and composition for electrodeposition of bright decorative chromium. More particularly, it relates to a chromium plating process characterized by highly satisfactory coverage of low current density areas.

As is well known to those skilled-in-the-art, chromium may be plated onto various basis metals. During chromium plating, it has been found that the coverage may not be completely satisfactory in low current density areas (typically below about 3–4 a.s.d.) and these areas may frequently receive little or no plate at all. Prior attempts to remedy this defect have included the use of auxiliary anodes; while this step may give some improvement, the disadvantages thereof are numerous and well known. Typically the burden of properly positioning the required anodes is undesirable and the cost of maintaining them on plating racks is very high.

Other techniques which have been tried include the use of various additives in the baths, but these additives have either been unable to give the desired result or have concurrently contributed some additional defect to the plate or to the process. Such defects may include the production of a blotching plate containing passivity spots, or result in an undesirably high degree of anode corrosion. Corrosion of lead anodes in chromium plating systems is undesirable in that a massive sludge is formed on the bottom of the tank; and the lead anodes are eaten away and must be replaced at regular intervals. Because of these problems, it is well recognized that prior art attempts to attain high coverage over the entire surface of the cathode and particularly in the areas of low current density have not been completely successful.

It is an object of this invention to provide a process for electrodepositing bright decorative chromium plate, characterized by its high coverage of low current density areas. Other objects will be apparent to those skilled-in-the-art on inspection of the following description.

## 2

In accordance with certain of its aspects, the process of this invention, characterized by high coverage and by high throwing power, for electrodepositing a bright decorative chromium plate onto a basis metal may comprise maintaining an aqueous hexavalent chromium plating bath containing chromic acid and sulfate in ratio of 125–550:1, and at least about 25 grams per liter of an anion of a halogenated organic carboxylic acid having at least three carbon atoms; and electrodepositing a chromium plate from said bath onto said basis metal as cathode in said bath.

The chromium plating bath which may be employed in practice of this invention in an aqueous solution containing 150 g./l.–500 g./l., typically 250 g./l.–400 g./l., say 250 g./l. of chromic acid  $\text{CrO}_3$  and 0.4 g./l.–3.3 g./l., say 1.2 g./l. of sulfate ion  $\text{SO}_4^{2-}$ , typically added as sodium sulfate. In practice of this invention, the ratio of  $\text{CrO}_3:\text{SO}_4^{2-}$  may preferably be maintained at 125–550:1, typically 200–300:1, say 250:1.

It is a particular feature of this invention that the novel results may be attained (a) in a standard, non-self regulating bath as described supra or (b) in a mixed catalyst bath or (c) in a self-regulating bath. A typical mixed catalyst bath which may be employed may contain 150–500 g./l., typically 250–400 g./l., say 250 g./l. of chromic acid  $\text{CrO}_3$  and 0.05–2.0 g./l., say 0.6 g./l. of sulfate  $\text{SO}_4^{2-}$  ion; and 0.05–2.0 g./l., say 0.6 g./l. of silicofluoride  $\text{SiF}_6^{2-}$  ion. It will be noted that the ratio as the term is used in this application refers to the ratio



wherein each of the quantities is expressed in grams. Other fluorides, including complex fluorides may be employed. When no other fluoride such as  $\text{SiF}_6^{2-}$  is present, the ratio may become



In practice, the ratio of  $\text{CrO}_3$  to  $\text{SO}_4^{2-}$  plus  $\text{SiF}_6^{2-}$  may preferably be maintained at 125–550:1, typically 200–300:1, say 250:1. In the specification and claims, the ratio may, for convenience, be referred to as the ratio of chromic acid to sulfate; but it will be understood that the ratio as so designated may include as equivalent to sulfate, other inorganic ions including fluoride ions such as the silicofluoride ion, the fluoborate ion, the fluotitanate ion, etc. Thus the designation "chromic acid to sulfate" includes chromic acid to sulfate plus other fluoride such as silicofluoride if and when the latter is present.

This invention may also be used in a self-regulating bath, e.g. of the sulfate type, which may contain 150–500 g./l., typically 250–400 g./l., say 250 g./l. of chromic acid; and 0.6–10 g./l., say 5 g./l., of strontium sulfate; plus optionally an additionally strontium compound source of excess strontium ion, such as strontium hydroxide, strontium chromate, etc. in amounts to provide 0–12 g./l., say 4.5 g./l. of strontium ion,  $\text{Sr}^{2+}$ . The ratio of  $\text{CrO}_3$  to  $\text{SO}_4^{2-}$  may preferably be maintained at 125–550:1, typically 200–300:1, say 250:1.

The halogenated organic carboxylic acids which may be added, either as such or e.g. as their anhydrides or salts (typically the sodium salt), to chromium plating baths in practice of this invention may typically include:

- (a) monohalogenated aliphatic monocarboxylic acids having at least three carbon atoms,
- (b) polyhalogenated aliphatic monocarboxylic acids having at least three carbon atoms,
- (c) monohalogenated aliphatic polycarboxylic acids having at least three carbon atoms,

- (d) polyhalogenated aliphatic polycarboxylic acids having at least three carbon atoms,
- (e) monohalogenated aromatic monocarboxylic acids having at least three carbon atoms,
- (f) monohalogenated aromatic polycarboxylic acids having at least three carbon atoms,
- (g) polyhalogenated aromatic monocarboxylic acids having at least three carbon atoms, and
- (h) polyhalogenated aromatic polycarboxylic acids having at least three carbon atoms.

Typical illustrative monohalogenated aliphatic monocarboxylic acids having at least three carbon atoms which may be employed may include:

- 2-chloropropionic acid
- 3-bromopropionic acid
- 3-iodopropionic acid
- 2-chlorobutanoic acid
- chloropivalic acid (monochlorinated tertiary pentanoic acid)
- 2-chloropentanoic acid

Typical illustrative polyhalogenated aliphatic monocarboxylic acids having at least three carbon atoms which may be employed may include:

- 2,2-dichloropropionic acid
- 2,2,3-trichloropropionic acid
- pentafluoropropionic acid

Typical illustrative monohalogenated aliphatic dicarboxylic acids having at least three carbon atoms which may be employed may include:

- chloromalonic acid
- 2-chlorosuccinic acid
- 2-bromosuccinic acid
- 2-chloroadipic acid

Typical illustrative polyhalogenated aliphatic dicarboxylic acids which may be employed may include:

- 2,2-dichlorosuccinic acid
- 2,2-dichloroadipic acid
- tetrachlorosuccinic acid
- 2,3-dibromosuccinic acid
- 3,3-diodosuccinic acid
- 3,4-dichloroadipic acid

Typical illustrative monohalogenated aromatic monocarboxylic acids which may be employed may include:

- 3-chloro-4-sulfobenzoic acid
- 3-bromo-4-sulfobenzoic acid

Typical illustrative monohalogenated aromatic dicarboxylic acids which may be employed may include:

- 4-chlorophthalic acid
- 2-bromoterephthalic acid

Typical illustrative polyhalogenated aromatic monocarboxylic acids which may be employed may include:

- 3,5-dichloro-4-sulfobenzoic acid
- 3,6-dibromo-4-sulfobenzoic acid

Typical illustrative polyhalogenated aromatic dicarboxylic acids which may be employed may include:

- 3,4-dichlorophthalic acid
- 3,4-dibromophthalic acid
- 4,5-dichlorophthalic acid

Other acids falling within the scope of this invention will be apparent to those skilled-in-the-art.

The preferred acids include halogenated aliphatic dicarboxylic acids having at least three carbon atoms and most preferably a halosuccinic acid such as 2-chlorosuccinic acid or 2,2-dichlorosuccinic acid or a halo adipic acid such as 3,4-dichloroadipic acid.

In practice of this invention, the carboxylic acid is added to the electroplating bath in amounts from 25 g./l.

up to the maximum practical concentration such as saturation, and preferably from 25 to 100 g./l. For many purposes the concentration may be in the narrower range from 25 to 50 g./l. The acids employed will preferably be those having a solubility in the plating bath within these ranges. Solubilizing substituents such as sulfo groups may be included in the carboxylic acid in order to increase solubility in the plating bath.

A typical composition which may be premixed, and added to a water solution in which the concentration of  $\text{SO}_4^{2-}$  ion and components including, e.g.,  $\text{SiF}_6^{2-}$ , may be adjusted separately, may include the compositions indicated in Tables I and II below (here as elsewhere, unless otherwise indicated, all parts are parts by weight). It will be apparent that these compositions, like other chromic acid - containing compositions, should preferably be formed, maintained, and stored in a manner to minimize contact with extraneous organic compositions and materials; and preferably they will be formed, stored, and maintained at temperature below 80° C. It will also be apparent that in compositions hereinafter designated as containing "halo-organic acid," halo-organic acid containing at least three carbon atoms is intended and equivalent amounts of anhydride, salt, etc. may be employed, thus yielding appropriate amounts of the desired ion.

TABLE I

| Component         | Max-<br>imum | Min-<br>imum | Preferred A | Preferred B |
|-------------------|--------------|--------------|-------------|-------------|
| $\text{CrO}_3$    | 500          | 150          | 250         | 400         |
| Halo-organic acid | 100          | 25           | 30          | 40          |

A preferred composition may include:

TABLE II

| Component                  | Max-<br>imum | Min-<br>imum | Preferred A | Preferred B |
|----------------------------|--------------|--------------|-------------|-------------|
| $\text{CrO}_3$             | 500          | 150          | 250         | 400         |
| 2,2-dichloro succinic acid | 100          | 25           | 30          | 40          |

The halo-organic acid may be added as such, as the anhydride, or as the salt, typically as the sodium salt. In the preferred embodiment, the additive may be admixed with the other ingredients to be used to make up the bath. Typically such a composition may include:

TABLE III

| Component                       | Max-<br>imum | Min-<br>imum | Preferred A | Preferred B |
|---------------------------------|--------------|--------------|-------------|-------------|
| $\text{CrO}_3$                  | 500          | 150          | 250         | 400         |
| $\text{SO}_4^{2-}$ <sup>1</sup> | 3.3          | 0.4          | 1.0         | 1.9         |
| Halo-organic acid               | 100          | 25           | 30          | 40          |

<sup>1</sup> Typically supplied as, e.g., sodium sulfate.

A specific self-regulating composition may include:

TABLE IV

| Component                 | Max-<br>imum | Min-<br>imum | Preferred A | Preferred B |
|---------------------------|--------------|--------------|-------------|-------------|
| $\text{CrO}_3$            | 500          | 150          | 250         | 400         |
| $\text{SrSO}_4$           | 10           | 4            | 4           | 8           |
| $\text{SrCrO}_4$          | 28           | 0            | 4.5         | 0           |
| 2,2-dichlorosuccinic acid | 100          | 25           | 30          | 40          |

A typical mixed catalyst composition may include:

TABLE V

| Component                        | Max-<br>imum | Min-<br>imum | Preferred A | Preferred B |
|----------------------------------|--------------|--------------|-------------|-------------|
| $\text{CrO}_3$                   | 500          | 150          | 250         | 400         |
| $\text{SO}_4^{2-}$ <sup>1</sup>  | 2.0          | 0.05         | 0.5         | 1.3         |
| $\text{SiF}_6^{2-}$ <sup>2</sup> | 2.0          | 0.05         | 0.5         | 0.7         |
| Halo-organic acid                | 100          | 25           | 30          | 40          |

<sup>1</sup> Typically added as sodium sulfate.

<sup>2</sup> Typically added as sodium silico fluoride.

A preferred mixed catalyst composition may include:

TABLE VI

| Component                       | Max-<br>imum | Min-<br>imum | Preferred A | Preferred B |
|---------------------------------|--------------|--------------|-------------|-------------|
| CrO <sub>3</sub> .....          | 500          | 150          | 250         | 400         |
| Sodium sulfate.....             | 3.0          | 0.075        | 0.75        | 1.9         |
| Sodium silicofluoride.....      | 2.7          | 0.065        | 0.65        | 0.9         |
| 2,2'-dichlorosuccinic acid..... | 100          | 25           | 30          | 40          |

A typical self-regulating composition having both sulfate and silicofluoride may include:

TABLE VII

| Component                            | Max-<br>imum | Min-<br>imum | Preferred A | Preferred B |
|--------------------------------------|--------------|--------------|-------------|-------------|
| CrO <sub>3</sub> .....               | 500          | 150          | 250         | 400         |
| SO <sub>4</sub> <sup>2-</sup> .....  | 2.0          | 0.05         | 0.5         | 1.3         |
| SiF <sub>6</sub> <sup>2-</sup> ..... | 2.0          | 0.05         | 0.5         | 0.7         |
| Sr <sup>++</sup> .....               | 9            | 0.2          | 5.0         | 2.6         |
| K <sup>+</sup> .....                 | 27           | 6.0          | 15          | 27          |
| Halo-organic acid.....               | 100          | 25           | 30          | 40          |

A preferred self-regulating composition may include:

TABLE VIII

| Component                                           | Max-<br>imum | Min-<br>imum | Preferred A | Preferred B |
|-----------------------------------------------------|--------------|--------------|-------------|-------------|
| CrO <sub>3</sub> .....                              | 500          | 150          | 200         | 325         |
| SrSO <sub>4</sub> .....                             | 8            | 0.1          | 2.0         | 4.0         |
| K <sub>2</sub> SiF <sub>6</sub> .....               | 6            | 0.75         | 2.0         | 3.5         |
| SrCrO <sub>4</sub> .....                            | 15           | 0            | 9           | 6           |
| K <sub>2</sub> Cr <sub>2</sub> O <sub>7</sub> ..... | 100          | 25           | 75          | 100         |
| 2,2-dichlorosuccinic acid.....                      | 100          | 25           | 30          | 40          |

The baths useful in practice of this invention may be formed by dissolving the above compositions in aqueous medium to form baths containing e.g. 150-500 g./l. of CrO<sub>3</sub> and corresponding quantities of the other components.

It is found that particularly outstanding results, in terms of handleability, packaging, ease of manufacture, as well as maximum coverage and brilliance of chromium deposit accompanied by a minimum of lead anode corrosion may be obtained when in the compositions of Tables I, III, V, and VII, the halo-organic acid is an aliphatic dicarboxylic acid having at least three carbon atoms; and such compositions are most highly preferred, because of their peculiarly unexpected superiority.

The baths of this invention which may be employed to readily and conveniently electrodeposit chromium plate, are characterized by high coverage and by high throwing power. These baths may be used to deposit chromium onto any basis metal. It is a particular feature of this invention that outstanding results may be obtained when the basis metal is a metal having an atomic number of 24-30. Typical of such basis metals are chromium, manganese, iron, cobalt, nickel, copper, and zinc. Mixtures or alloys of these metals may be plated—typically brass, stainless steel, etc. The preferred basis metal may be nickel, and preferably active nickel.

The preferred active nickel basis metal may be attained by electrodeposition of nickel onto a suitable substrate metal (such as iron).

Active nickel may be nickel which is highly receptive to the deposition thereon of a bright clear decorative plate and which has a surface which may be free of nickel compounds such as the oxide. Typically nickel may be active when freshly plated onto a cathode. If not already active, the nickel may be rendered active by cathodic or other reducing treatment prior to the deposition of chromium plate thereon. Preferably this may be effected by maintaining the nickel as cathode in an aqueous electrolyte solution, preferably containing an acid. The preferred acids for use in either electrolytic or non-electrolytic techniques may include acids such as the common mineral acids e.g. hydrochloric acid or sulfuric acid, etc. When the aqueous electrolyte solution is other than acid, it may preferably be followed by an acid dip.

It has been found when the high ratio baths of this invention are used to plate chromium onto bright nickel

basis metal that it is advantageous to activate the bright nickel by applying to the cathode to be plated in the bath, a low voltage applied thereto at a time less than about five seconds after immersion and preferably to apply the voltage prior to immersion of the cathode. The low voltage may be sufficient to produce a cathode current density up to about 0.25-0.5 times the plating current density. Then the current density may be raised to its full operating value. This technique makes a bright nickel surface more receptive to the deposit of bright chromium from the baths of this invention.

The bath may be preferably at temperature of 30°-60° C., say 35°-50° C. A preferred cathode current density may be 0.3-40 amperes per square decimeter (a.s.d.) most preferably 0.5-20 a.s.d. Plating may be carried out with air or mechanical agitation for any time to obtain a desired thickness, but for decorative plate it is usually 1-10 minutes; and typically about five minutes may suffice.

During plating in accordance with the process of this invention, there is unexpectedly and surprisingly no appreciable loss of the halo-organic acid by decomposition over extended periods of time. For example, in tests, 2,2-dichlorosuccinic acid was found still to function satisfactorily after plating had been carried out for 110 ampere hours per liter and even longer.

At the conclusion of the plating time, the cathode will be found to be covered to a remarkable degree with clear, bright, decorative chromium plate. It is a particular feature of this invention that the plate is unexpectedly characterized by its high coverage without the need for conforming anodes. For example, articles containing deep recesses such as zinc based die cast automotive dashboard trim may be plated by the process of this invention (with no conforming anode) to unexpectedly yield a bright, uniform plate on both high and low current density areas. This has not heretofore been possible.

The plate produced by the novel process of this invention may be found to be highly satisfactory with respect to its unusually bright, decorative appearance and its resistance to corrosion.

In the following series of illustrative examples, chromium was electrodeposited onto a 100 mm. nickel-plated brass panel in a standard Hull Cell at 49° C. for five minutes and three amperes. A standard stock bath containing 300 g./l. chromic acid and 1.3 g./l. of sulfate (added as sulfuric acid) was employed. The halo-organic acid was added in the amount (in g./l.) indicated. At the end of the test, the Hull Cell panel was inspected and the distance across the panel bearing a plate of clear bright chromium was measured in millimeters.

TABLE IX

|          | Acid added                         | G./l. | Coverage,<br>mm. |
|----------|------------------------------------|-------|------------------|
| Example: |                                    |       |                  |
| 1        | None.....                          | 23    | 57               |
| 2        | 2,2-dichlorosuccinic acid.....     | 23    | 77               |
| 3        | do.....                            | 29    | 77               |
| 4        | do.....                            | 33    | 79               |
| 5        | Tetrachlorosuccinic acid.....      | 25    | 75               |
| 6        | 2,3-dibromosuccinic acid.....      | 25    | 70               |
| 7        | 3,4-dichloro adipic acid.....      | 25    | 79               |
| 8        | 2-chloropropionic acid.....        | 25    | 73               |
| 9        | do.....                            | 32    | 77               |
| 10       | do.....                            | 45    | 76               |
| 11       | 3-chloropropionic acid.....        | 25    | 76               |
| 12       | 2,2-dichloropropionic acid.....    | 36    | 73               |
| 13       | 2,2,3-trichloropropionic acid..... | 30    | 78               |
| 14       | 3-bromopropionic acid.....         | 25    | 77               |

In the following series of illustrative examples the stock bath and the plating conditions were the same as in the previous examples, except that electrodeposition was conducted at 43° C.

TABLE X

|          | Acid added         | G./l. | Coverage, mm. |
|----------|--------------------|-------|---------------|
| Example: | None               |       | 58            |
| 15.      | Chloropivalic acid | 25    | 80            |

In the following series of examples, chromium was electrodeposited onto Hull Cell panels at 43° C. for five minutes and three amperes from a series of mixed catalyst baths containing 400 g./l. of chromic acid and sulfate, silicofluoride and halo-organic acid in the amounts (in g./l.) indicated.

TABLE XI

|          | SO <sub>4</sub> <sup>2-</sup> , g./l. | SiF <sub>6</sub> <sup>2-</sup> , g./l. | Acid added                    | Acid, g./l. | Coverage, mm. |
|----------|---------------------------------------|----------------------------------------|-------------------------------|-------------|---------------|
| Example: |                                       |                                        |                               |             |               |
| 17.      | 0.667                                 | 0.667                                  | None                          |             | 55            |
| 18.      | 0.667                                 | 0.667                                  | 2,3-dibromosuccinic acid      | 25          | 70            |
| 19.      | 0.64                                  | 0.32                                   | None                          |             | 55            |
| 20.      | 0.64                                  | 0.32                                   | 2,2,3-trichloropropionic acid | 25          | 72            |
| 21.      | 1.28                                  | 0.64                                   | None                          |             | 54            |
| 22.      | 1.28                                  | 0.64                                   | 3,4-dichloroadipic acid       | 25          | 76            |

In the following series of examples, chromium was electrodeposited onto Hull Cell panels at 43° C. for five minutes and three amperes from a series of self-regulating baths containing 425 g./l. of chromic acid, 8.0 g./l. of strontium sulfate. The halo-organic acid was added in the amount (in g./l.) indicated.

TABLE XII

|          | Acid added                | G./l. | Coverage, mm. |
|----------|---------------------------|-------|---------------|
| Example: |                           |       |               |
| 23.      | None                      |       | 52            |
| 24.      | 2-chloropropionic acid    | 40    | 78            |
| 25.      | do                        | 160   | 79            |
| 26.      | 2,3-dibromo-succinic acid | 25    | 70            |

From Examples 1, 15, 17, and 23, it may be observed that with no halo-organic acid added, the panel was respectively covered for a distance of 57 mm., 58 mm., 55 mm., and 52 mm. and these may be considered control examples for the examples which follow. As the 2,2-dichlorosuccinic acid concentration increased, e.g. from 25 g./l. to 33 g./l., the coverage increased to as high as 79 mm. A difference of 2-3 mm. or more may be considered significant. Example 4 was carried out in a bath which had been functioning for 40 ampere hours per liter, this indicating that the system including 2,2-dichlorosuccinic acid was stable over an extended period. Similarly Example 8 was carried out after a life test for 65 ampere hours per liter. Thus, it will be apparent from these examples, that practice of this invention permits attainment of a high degree of coverage.

It is also a feature of the baths of this invention that the preferred halo-organic carboxylic acids herein disclosed are characterized by their substantially decreased degree of attack of lead anodes. This latter may be observed for example by immersing lead in two baths containing 350 g./l. CrO<sub>3</sub>, and 1.4 g./l. SO<sub>4</sub><sup>2-</sup>. The baths, together with the indicated additive, may be left to stand for 22 hours at 49° C., then electrolyzed at 15 a.s.d. for one hour and then left to stand again for 65 hours at approximately 21° C. with the following results:

TABLE XIII

|          | Additive                 | G./l. | Loss of weight, grams |
|----------|--------------------------|-------|-----------------------|
| Example: |                          |       |                       |
| 27.      | 3, 4-dichloroadipic acid | 25    | 0.237                 |
| 28.      | Trichloroacetic acid     | 25    | 5.347                 |

Thus it will be seen that the loss in weight of the lead is much lower (only 4.4% as much) when the baths of this invention are used than when a bath is used containing trichloroacetic acid.

It had been believed that the organic compounds used in practice of this invention would be quickly oxidized in the presence of chromic acid, a well known oxidizing agent and thus be substantially inoperable. It is however a particular feature of the baths of this invention containing halo-organic acids such as 2,2-dichlorosuccinic acid, that they may unexpectedly be stable over extended periods of operation.

In order to demonstrate the stability of the baths of this invention under severe operating conditions, a bath may be prepared containing 300 g./l. CrO<sub>3</sub>, 1.3 g./l. SO<sub>4</sub><sup>2-</sup>, and 75 g./l. of 2,2-dichlorosuccinic acid. The bath may be heated to 93° C. and electrolyzed at a high current density of 60 a.s.d. (94 amperes per liter of solution). Electrolysis may continue over four hours at 93° C. using a lead anode and a steel cathode. At the conclusion of the test, the voltage drop across the bath may be noted and found to be unchanged. This indicates that no trivalent or reduced chromium is present and thus that no 2,2-dichlorosuccinic acid had been oxidized. As is well known to those skilled-in-the-art, acids such as citric acid, tartaric acid, oxalic acid, etc. (which are not within the scope of this invention) would oxidize substantially immediately on contact with chromium baths.

Although the outstandingly high coverage herein noted may be attained by the several halo-acids set forth, it may be found that halogenated dicarboxylic aliphatic acids having at least three carbon atoms are unexpectedly superior in that they permit operation at desirably high ratio (of e.g. CrO<sub>3</sub> to SO<sub>4</sub><sup>2-</sup>) with high coverage and minimum attack on anodes. For example, such acids typified by 3,4-dichloroadipic acids, may give maximum coverage, with a lead anode corrosion which is unexpectedly and significantly less than that attained when acids such as trichloroacetic acid are used. Furthermore, loss of acid such as halogenated adipic acids from plating baths may be found to be considerably less from evaporation than loss of e.g. halogenated acetic acid from these baths. These factors, *inter alia*, dictate that the acids having at least three carbon atoms permit attainment of unexpectedly superior advantages.

It is a particularly outstanding feature of the preferred embodiment of this invention that when halogenated dicarboxylic acids such as halogenated succinic acid and halogenated adipic acid are used that the coverage with chromium plate is extremely high, and interior portions of the cathodes are uniformly covered by a bright, decorative plate. Furthermore, the color, brilliance, and clarity of the plate on the open or exposed areas is far superior to that attained by use of the best prior art baths. The process is further characterized by freedom from anode attack and by substantially lower tendency toward undesirable development of "chromate-film" on low current density areas which would decrease the appearance and attractiveness of decorative plate.

Although this invention has been illustrated by reference to specific examples, numerous changes and modi-

ifications thereof which clearly fall within the scope of the invention will be apparent to those skilled-in-the-art.

We claim:

1. The process characterized by high coverage and by high throwing power for electrodepositing a bright decorative chromium plate onto a basis metal which comprises maintaining an aqueous hexavalent chromium plating bath containing chromic acid and sulfate in ratio of 125-550:1 and at least about 25 grams per liter of an anion of a halogenated organic acid of the group consisting of aliphatic and aromatic monocarboxylic and dicarboxylic acids having at least three carbon atoms, and electrodepositing a bright decorative chromium plate from said bath onto said basis metal as cathode in said bath.

2. The process characterized by high coverage and by high throwing power for electrodepositing a bright decorative chromium plate onto a basis metal which comprises maintaining an aqueous hexavalent chromium plating bath containing chromic acid and sulfate in ratio of 125-550:1 and at least about 25 grams per liter of an anion of a halogenated aliphatic dicarboxylic acid having at least three carbon atoms, and electrodepositing a bright decorative chromium plate from said bath onto said basis metal as cathode in said bath.

3. The process as claimed in claim 2 for electrodepositing a bright decorative chromium plate onto a basis metal wherein said acid is a chlorinated adipic acid.

4. The process as claimed in claim 2 for electrodepositing a bright decorative chromium plate onto a basis metal wherein said acid is a chlorinated succinic acid.

5. The process as claimed in claim 2 for electrodepositing a bright decorative chromium plate onto a basis metal wherein said halogenated organic acid is present in said bath in amount of 25 to 100 grams per liter.

6. The process characterized by high coverage and by high throwing power for electrodepositing a bright decorative chromium plate onto a basis metal which comprises maintaining an aqueous chromium plating bath containing 150-500 g./l. chromic acid and 0.4-3.3 g./l. sulfate ion, and a ratio of chromic acid to sulfate of 125-550:1, and from 25 to 100 g./l. of an anion of a halogenated organic acid of the group consisting of aliphatic and aromatic monocarboxylic and dicarboxylic acids having at least three carbon atoms, and electrodepositing a bright decorative chromium plate from said bath onto said basis metal as cathode in said bath.

7. The process characterized by high coverage and by high throwing power for electrodepositing a bright decorative chromium plate onto a basis metal which comprises maintaining an aqueous mixed-catalyst chromium plating bath containing 150-500 g./l. of chromic acid, 0.05-2.0 g./l. of sulfate ion and 0.05-2.0 of silicofluoride ion, the ratio of chromic acid to sulfate ion plus silicofluoride ion being 125-550:1, and 25-100 g./l. of an anion of a halogenated organic acid of the group consisting of aliphatic and aromatic monocarboxylic and dicarboxylic acids having at least three carbon atoms, and electrodepositing a bright decorative chromium plate from said bath onto said basis metal as cathode in said bath.

8. The process characterized by high coverage and by high throwing power for electrodepositing a bright decorative chromium plate onto a basis metal which comprises maintaining an aqueous self-regulating chromium plating bath containing 150-500 g./l. of chromic acid, 0.6-10 g./l. of strontium sulfate and 0-12 g./l. of excess strontium ion, the ratio of chromic acid to sulfate being 125-550:1 and 25-100 g./l. of an anion of a halogenated organic acid of the group consisting of aliphatic and aromatic monocarboxylic and dicarboxylic acids having at least three carbon atoms, and electrodepositing a bright decorative chromium plate from said bath onto said basis metal as cathode in said bath.

9. A composition for addition to an aqueous medium to form a bath for the electrodeposition of bright

chromium plate onto a basis metal consisting essentially of the following components in the designated parts by weight:

| Component              | Maximum | Minimum |
|------------------------|---------|---------|
| Chromic acid.....      | 500     | 150     |
| Sulfate ion.....       | 3.3     | 0.4     |
| Halo-organic acid..... | 100     | 25      |

the ratio of chromic acid to sulfate being 125-550:1 and the halo-organic acid being a halogenated organic acid selected from the group consisting of aliphatic and aromatic monocarboxylic and dicarboxylic acids having at least three carbon atoms.

10. A composition as claimed in claim 9 for addition to an aqueous medium to form a bath for the electrodeposition of bright chromium plate onto a basis metal wherein said halo-organic acid is 3,4-dichloroadipic acid.

11. A composition as claimed in claim 9 for addition to an aqueous medium to form a bath for the electrodeposition of bright chromium plate onto a basis metal wherein said halo-organic acid is 2,2'-dichlorosuccinic acid.

12. A composition for addition to an aqueous medium to form a bath for the electrodeposition of bright chromium plate onto a basis metal consisting essentially of the following components in the designated parts by weight:

| Component               | Maximum | Minimum |
|-------------------------|---------|---------|
| Chromic acid.....       | 500     | 150     |
| Sulfate ion.....        | 2.0     | 0.05    |
| Silicofluoride ion..... | 2.0     | 0.05    |
| Halo-organic acid.....  | 100     | 25      |

the ratio of chromic acid to sulfate plus silicofluoride being 125-550:1 and the organic acid being a halogenated organic acid selected from the group consisting of aliphatic and aromatic monocarboxylic and dicarboxylic acids having at least three carbon atoms.

13. A composition for addition to an aqueous medium to form a bath for the electrodeposition of bright chromium plate onto a basis metal consisting essentially of the following components in the designated parts by weight:

| Component                            | Maximum | Minimum |
|--------------------------------------|---------|---------|
| CrO <sub>3</sub> .....               | 500     | 150     |
| SO <sub>4</sub> <sup>2-</sup> .....  | 2.0     | 0.05    |
| SiF <sub>6</sub> <sup>2-</sup> ..... | 2.0     | 0.05    |
| Sr <sup>2+</sup> .....               | 9       | 0.2     |
| K <sup>+</sup> .....                 | 27      | 6.0     |
| Halo-organic acid.....               | 100     | 25      |

the ratio of chromic acid to sulfate plus silicofluoride being 125-550:1 and the halo-organic acid being a halogenated organic acid selected from the group consisting of aliphatic and aromatic monocarboxylic and dicarboxylic acids having at least three carbon atoms.

14. A chromium plating solution for the electrodeposition of bright chromium plate onto a basis metal which comprises an aqueous solution of chromic acid and sulfate in ratio of 125-550:1, and at least 25 grams per liter of an anion of a halogenated organic acid of the group consisting of aliphatic and aromatic monocarboxylic and dicarboxylic acids having at least 3 carbon atoms.

15. A chromium plating solution as claimed in claim 14 for the electrodeposition of bright chromium plate onto a basis metal wherein said halogenated organic carboxylic acid is 2,2-dichlorosuccinic acid.

16. A chromium plating solution as claimed in claim 14 for the electrodeposition of bright chromium plate onto a basis metal wherein said halogenated organic acid is present in amount of 25 to 100 g./l.

17. A chromium plating solution for the electrodeposition of bright chromium plate onto a basis metal which comprises an aqueous solution of 150-500 g./l. of chromic acid, 0.05-2.0 g./l. of sulfate ion and 0.05-2.0 g./l. of silicofluoride ion, the ratio of chromic acid to sulfate

plus silicofluoride being 125-550:1, and 25-100 g./l. of a halogenated organic acid of the group consisting of aliphatic and aromatic monocarboxylic and dicarboxylic acids having at least 3 carbon atoms.

18. A chromium plating solution for the electrodeposition of bright chromium plate onto a basis metal which comprises an aqueous solution of 150-500 g./l. of chromic acid, 0.6-10 g./l. of strontium sulfate, the ratio of chromic acid to sulfate being 125-550:1, and 0-12 g./l. of excess strontium ion, and 25-100 g./l. of an anion of a halogenated organic acid of the group consisting of aliphatic and aromatic monocarboxylic and dicarboxylic acids having at least 3 carbon atoms.

19. The process characterized by high coverage and by high throwing power for electrodepositing a bright decorative chromium plate onto a basis metal which comprises maintaining an aqueous chromium plating bath containing 150-500 g./l. chromic acid and 0.4-3.3 g./l. sulfate ion, and a ratio of chromic acid to sulfate of 125-550:1, and from 25 to 100 g./l. of an anion of a halogenated aliphatic dicarboxylic acid having at least three carbon atoms, and electrodepositing a bright decorative chromium plate from said bath onto said basis metal as cathode in said bath.

20. The process characterized by high coverage and by high throwing power for electrodepositing a bright decorative chromium plate into a basis metal which comprises maintaining an aqueous mixed-catalyst chromium plating bath containing 150-500 g./l. of chromic acid, 0.05-2.0 g./l. of sulfate ion and 0.05-2.0 g./l. of silicofluoride ion, the ratio of chromic acid to sulfate ion plus silicofluoride ion being 125-550:1, and 25-100 g./l. of an anion of a halogenated organic dicarboxylic acid having at least three carbon atoms, and electrodepositing a bright decorative chromium plate from said bath onto said basis metal as cathode in said bath.

21. The process characterized by high coverage and by high throwing power for electrodepositing a bright decorative chromium plate onto a basis metal which comprises maintaining an aqueous self-regulating chromium plating bath containing 150-500 g./l. of chromic acid, 0.6-10 g./l. of strontium sulfate and 0-12 g./l. of excess strontium ion, the ratio of chromic acid to sulfate of 125-550:1 and 25-100 g./l. of an anion of a halogenated aliphatic dicarboxylic acid having at least three carbon atoms; and electrodepositing a bright decorative chromium plate from said bath onto said basis metal as cathode in said bath.

22. A composition for addition to an aqueous medium to form a bath for the electrodeposition of bright chromium plate onto a basis metal consisting essentially of the following components in the designated parts by weight:

| Component              | Maximum | Minimum |
|------------------------|---------|---------|
| Chromic acid.....      | 500     | 150     |
| Sulfate ion.....       | 3.3     | 0.4     |
| Halo-organic acid..... | 100     | 25      |

the ratio of chromic acid to sulfate being 125-550:1 and the halo-organic acid being a halogenated aliphatic dicarboxylic acid having at least three carbon atoms.

23. A composition for addition to an aqueous medium to form a bath for the electrodeposition of bright chromium plate onto a basis metal consisting essentially of

5

the following components in the designated parts by weight:

| Component               | Maximum | Minimum |
|-------------------------|---------|---------|
| Chromic acid.....       | 500     | 150     |
| Sulfate ion.....        | 2.0     | 0.05    |
| Silicofluoride ion..... | 2.0     | 0.05    |
| Halo-organic acid.....  | 100     | 25      |

the ratio of chromic acid to sulfate plus silicofluoride being 125-550:1 and the organic acid being a halogenated aliphatic dicarboxylic acid having at least three carbon atoms.

24. A composition for addition to an aqueous medium to form a bath for the electrodeposition of bright chromium plate onto a basis metal consisting essentially of the following components in the designated parts by weight:

| Component                            | Maximum | Minimum |
|--------------------------------------|---------|---------|
| CrO <sub>3</sub> .....               | 500     | 150     |
| SO <sub>4</sub> <sup>2-</sup> .....  | 2.0     | 0.05    |
| SiF <sub>6</sub> <sup>2-</sup> ..... | 2.0     | 0.05    |
| Sr <sup>2+</sup> .....               | 9       | 0.2     |
| K <sup>+</sup> .....                 | 27      | 6.0     |
| Halo-organic acid.....               | 100     | 25      |

the ratio of chromic acid to sulfate plus silicofluoride being 125-550:1 and the halo-organic acid being a halogenated aliphatic dicarboxylic acid having at least three carbon atoms.

25. A chromium plating solution for the electrodeposition of bright chromium plate onto a basis metal which comprises an aqueous solution of chromic acid and sulfate in ratio of 125-550:1, and at least 25 grams per liter of an anion of 3,4-dichloroadipic acid.

26. A chromium plating solution for the electrodeposition of bright chromium plate onto a basis metal which comprises an aqueous solution of chromic acid and sulfate in ratio of 125-550:1, and at least 25 grams per liter of anion of 2,2'-dichlorosuccinic acid.

27. A chromium plating solution for the electrodeposition of bright chromium plate onto a basis metal which comprises an aqueous solution of 150-500 g./l. of chromic acid, 0.05-2.0 g./l. of sulfate ion and 0.05-2.0 g./l. of silicofluoride ion, the ratio of chromic acid to sulfate plus silicofluoride being 125-550:1, and 25-100 g./l. of a halogenated aliphatic dicarboxylic acid having at least 3 carbon atoms.

28. A chromium plating solution for the electrodeposition of bright chromium plate onto a basis metal which comprises 150-500 g./l. of chromic acid, 0.6-10 g./l. of strontium sulfate, the ratio of chromic acid to sulfate being 125-550:1, and 0-12 g./l. of excess strontium ion, and 25-100 g./l. of an anion of a halogenated aliphatic dicarboxylic acid having at least 3 carbon atoms.

55

#### References Cited

##### UNITED STATES PATENTS

|           |         |                      |        |
|-----------|---------|----------------------|--------|
| 2,623,847 | 12/1952 | Gilbert et al. ----- | 204-51 |
| 2,640,022 | 5/1953  | Stareck -----        | 204-51 |
| 3,248,310 | 4/1966  | Schaer -----         | 204-51 |
| 3,282,812 | 11/1966 | Brown et al. -----   | 204-51 |

JOHN H. MACK, Primary Examiner

G. L. KAPLAN, Assistant Examiner

50

60

65